

D. RAWSTRON.  
MOLDING AND CASTING REINFORCED BRAKE SHOES.  
APPLICATION FILED OCT. 5, 1909.  
**964,054.** Patented July 12, 1910.



WITNESSES:

*H. G. McMillan*  
*F. M. Kendrick*

*Fig. 5*

BY

INVENTOR:  
Donald Rawstron  
Bigout & Maybee  
ATTORNEYS.

# UNITED STATES PATENT OFFICE.

DONALD RAWSTRON, OF CHICAGO, ILLINOIS.

## MOLDING AND CASTING REINFORCED BRAKE-SHOES.

964,054.

Specification of Letters Patent. Patented July 12, 1910.

Application filed October 5, 1909. Serial No. 521,108.

*To all whom it may concern:*

Be it known that I, DONALD RAWSTRON, of the city of Chicago, State of Illinois, United States of America, have invented 5 certain new and useful Improvements in Molding and Casting Reinforced Brake-Shoes, of which the following is a specification.

This invention relates to the molding and 10 casting of brake shoes provided with tough metal reinforcing strips at the back and a separate tough metal hook-shaped attaching lug, and my object is to devise a process of molding such shoes which will insure that 15 the gape of the hook will always be exactly the same in every shoe cast.

I attain my object by adopting a particular arrangement of the hook and reinforcement and by following a process of molding 20 which may be briefly described as follows: The lug is formed with shoulders on its shank engaging the underside of the reinforcement. A suitable shape of pattern is employed to form in the cope of the flask a 25 recess for the reception of the lug and for a core which separates the jaw of the hook from the reinforcement. This core holds the hook up with its shoulders in contact with the reinforcement and accurately de- 30 terminates the gape of the hook.

Figure 1 is a longitudinal section of a molding box or flask prepared ready for the casting of a brake shoe. Fig. 2 is a cross section of the same adjacent to the 35 attaching lug. Fig. 3 is a perspective detail illustrating the relative positions of the end of the brake shoe, the lug, the reinforcement and the core forming the gape of the lug. Fig. 4 is a perspective detail of the pattern 40 used in molding the brake shoe. Fig. 5 is a plan view of the back of a brake shoe constructed in accordance with my invention.

In the drawings like letters of reference indicate corresponding parts in the different 45 figures.

The brake shoe itself comprises a cast metal body A, the reinforcing strips B of a tough or malleable metal, and the attaching lug C, also of tough or malleable metal.

50 The reinforcement is construed substantially as shown and described in U. S. Patent No. 725,587, dated April 14th, 1903, but,

of course, other forms of reinforcement at the back of the shoe might be employed for the purpose of the present invention. 55

The attaching lug C is hook-shaped being provided with the jaw D extending toward the middle of the shoe substantially parallel to the back. I form the lug C with the shoulders  $\alpha$  which engage the undersides of 60 the reinforcement B. This contact determines the maximum gap of the lug or hook.

In order to insure the gape being the same in every brake shoe cast I have devised the process hereinbefore partly described 65 and which I will now set out in detail.

A pattern is formed substantially as shown in Fig. 4, E forming the body of the shoe and F forming the recess for the reception of the attaching lug and a core used 70 in settling the gape of the lug.

In Figs. 1 and 2 I show the molding box or flask, G being the cope and H the drag. The shoe is molded in the flask, the back being molded in the cope of the flask. After 75 the impression has been taken from the pattern, the cope is turned over and the lug C placed in the print ready to receive it. As already stated, the part F of the pattern forms the print for the projecting part of 80 the lug and for the core I. This core is separately formed and placed in position as indicated in Figs. 1-2 and 3 between the jaw D of the lug and the reinforcement which is in contact with the shoulders  $\alpha$ . 85 The reinforcement may be secured to the cope by nails in the ordinary manner and the parts of the flask placed together, as shown in Figs. 1 and 2.

It is evident that the core I insures that 90 in every brake shoe cast the jaw of the lug will be separated from the back of the shoe by a space having exactly the same depth in every shoe, consequently when the shoes have been cast in molds prepared as just 95 described all the lugs will be exactly the same in their gap, and the trouble now frequently experienced with ill fitting lugs will be entirely avoided.

What I claim as my invention is:—

100 A process of securing an attaching lug in a cast metal brake shoe provided with a reinforcement at its back, which consists in forming the lug with a shoulder adapted

2  
to engage the underside of the reinforcement, molding the shoe and forming a print for the external part of the lug and for a core to separate the jaw of the lug from the  
5 reinforcement, placing the lug and reinforcement in position and then pouring the mold in the ordinary manner, forming a core and inserting it in the print in the

mold to hold the shoulder on the lug in contact with the underside of the reinforcement. 10

Chicago, Illinois, this 27 day of September 1909.

DONALD RAWSTRON.

Signed in the presence of—

HERMAN F. BUNDE,

EUGENE C. HERMESTROFF.